

United States Patent [19]  
Schick

[11] 3,867,180  
[45] Feb. 18, 1975

[54] PRODUCT AND PROCESS

[75] Inventor: Mary Margaret Schick, Wilmington, Del.

[73] Assignee: E. I. du Pont de Nemours & Co., Wilmington, Del.

[22] Filed: May 24, 1973

[21] Appl. No.: 363,664

[52] U.S. Cl. 117/76 FB, 117/76 T, 117/104 R, 117/138.8 F, 117/140 A, 161/92, 161/155, 161/156

[51] Int. Cl. B44d 1/08, B44d 1/16

[58] Field of Search 117/140 A, 76 FB, 76 T, 117/98, 138.8 F, 104 R; 161/92, 155, 156; 252/8.7, 8.9

[56] References Cited

UNITED STATES PATENTS

|           |         |                |           |
|-----------|---------|----------------|-----------|
| 2,677,700 | 5/1954  | Jackson et al. | 252/8.9 X |
| 3,381,077 | 4/1968  | Bonner         | 264/321   |
| 3,402,070 | 9/1968  | Brudmann       | 117/138.8 |
| 3,461,026 | 8/1969  | Schick         | 161/154   |
| 3,485,711 | 12/1969 | Fish et al.    | 161/150   |
| 3,535,181 | 10/1970 | Yunan          | 156/181   |

OTHER PUBLICATIONS

Schick, Nonionic Surfactants, Pub. 1967 by Marcel Dekker, Inc., New York, pages 309, 310, 312, 320, 350-352.

Primary Examiner—Leon D. Rosdol  
Assistant Examiner—Harris A. Pitlick

[57] ABSTRACT

A process is disclosed for reducing the noise level created when a compressive load is placed on a bonded reticulated batt of randomly arranged pneumatic closed-cell foamed fibers so as to flex the fibers. The reduction is achieved by coating the batt, prior to coating it with an adhesive binder, with an anti-adhesive which is a selected polysiloxane, a selected polyoxyethylene polyoxypropylene glycol or a selected alkyl sodium sulfonate. The anti-adhesive prevents formation of weak bonds between the fiber and the adhesive which have been found to be the source of the noise (created when the weak bonds break) but does not prevent the formation of the usual strong bonds between the fiber and the adhesive.

5 Claims, No Drawings

## PRODUCT AND PROCESS

## FIELD OF THE INVENTION

This invention relates to the reduction of noise in fibrous cushioning structures when they are flexed under load. More specifically, this invention is directed to such noise-reduction in nonwoven batts of pneumatic foamed closed-cell fibers by coating the batts with a selected anti-adhesive prior to the application of an adhesive binder.

## BACKGROUND

Numerous types of foamed polymeric materials are used for cushioning applications. Among them are closed-cell microcellular foamed fibers in which the cells are inflated with an inflatant that is impermeant to the cell walls and thus is confined within the cells, making the fibers permanently pneumatically resilient. These fibers, referred to herein as "microcellular, inflated closed-cell pneumatic fibers", are made of synthetic organic polymers. They can be used to prepare reticulated batts in which the fibers are randomly arranged within the batt and contact one another frequently at crossover points. To aid dimensional stability these batts are usually treated with an adhesive binder. These preparations are described in U.S. Pat. Nos. 3,461,026; 3,485,711; 3,535,181; and 3,381,077, *inter alia*.

As stated above, to aid the dimensional stability of the batts, the batts are usually subjected to an adhesive binder which infiltrates the batt and binds the fibers therein at their crossover points. The batts are useful as cushioning structures for a variety of purposes, such as pillows or as an overlayer on mattress springs. However, when flexed under a load, these bonded batts emit an auditory signal, or noise, which is objectionable to the ear, being a crackling noise.

It is believed that the noise is due to the breaking of weak bonds between the fibers in the batts and the adhesive binder, and it has now been discovered that, by applying a mild anti-adhesive to the batt before the adhesive binder is applied, these weak bonds can be prevented from forming. Thus, the objectionable crackling heard when the batts are stressed under load can be reduced by the use of the anti-adhesive. A process involving its use comprises the process of this invention.

## SUMMARY OF THE INVENTION

This invention provides a process for reducing the noise in compressible fibrous structures when flexed under stress, which comprises:

spraying a reticulated batt of randomly arranged, microcellular, inflated closed-cell, pneumatic fibers of a synthetic organic polymer with between about 0.03 to about 5 percent by weight based on the weight of the fibers of an anti-adhesive composition comprising a polyoxyethylene polyoxypropylene polymethylsiloxane containing about 51% polyoxyethylene, a sodium alkylsulfonate of 22 to 24 carbon atoms, or a polyoxyethylene polyoxypropylene glycol containing about 80% polyoxyethylene. The polysiloxane can be obtained from Dow-Corning as DC 473 fluid; the glycol can be obtained from BASF-Wyandotte as "Pluronic".

The anti-adhesive is coated onto the batt, either by dipping the batt into an aqueous mixture containing it, or by spraying it onto the unbonded batt from an aqueous dispersion to a level between about 0.03 and 5%, preferably 0.05 and 0.3%, by weight of the anti-adhesive based on the batt. Spray application is preferred for continuous preparation of the batts of this invention. The aqueous dispersion may conveniently comprise 0.1-0.3% of the active ingredient. The batt should be sprayed with water prior to application of the coatings. Wetting aids in application of the coating.

The anti-adhesive coating applied need not be dried, although it can be if desired, for the adhesive binder may be applied immediately thereafter. The adhesive binder is conveniently applied by spraying it on the batt although dipping the batt, while supported between scrims, in a dispersion of the adhesive may be employed. The binder employed is a copolymer of ethylene and vinyl acetate containing 18-40% by weight po-

drying the coated batt.

## DESCRIPTION OF THE INVENTION

The batts used in the process of this invention are reticulated structures containing the microcellular, inflated closed-cell, pneumatic filaments laid down on top of one another to obtain numerous crossings of filament portions and penetration of portions of filaments at one thickness level into adjacent thickness levels. Individual filaments in the batt will vary in configuration from straight to curved to S shaped. An uncompressed batt may contain 3 to 4 oz./sq. yd. of the filaments. Ordinarily, the batts are obtained by laying the filaments down on a horizontal surface and building up layers until the desired thickness is obtained.

The fibers useful herein, as described above, may be prepared as disclosed in U.S. Pat. Nos. 3,375,211; 3,375,212; 3,503,907; 3,584,090 or 3,381,077. In general, the fibers are made from fiber-forming, organic polymers, especially polymers of ethylene terephthalate or vinyl chloride or copolymers predominantly comprising units of either of the foregoing and up to about 10% by weight of units derived from other compounds copolymerizable therewith.

In general, the fibers are formed by flash extrusion in which a solution of the polymer in a solvent is maintained at super atmospheric pressure and at a temperature above the boiling point of the solvent. By careful adjustment of conditions, as described in said patents, the microcellular, closed-cell fibers are obtained. The fibers are usually post-inflated, i.e., the inflatant is added to the cell interior to provide the inflated, pneumatic properties of the fiber. This inflation procedure is also described in the aforementioned U.S. patents. Generally, the fibers contain about  $10^5$  or more cells per cc of fiber and when inflated have a density of between about 0.008 and 0.05 gm./cc. In addition, the inflated fiber diameters can range from about 0.025 to 0.25 inch, preferably about .03 to about 0.10 inch.

The anti-adhesive used herein is a surface-active agent, and is a polyoxyethylene polyoxypropylene polymethylsiloxane containing about 51% polyoxyethylene, a sodium alkylsulfonate of 22 to 24 carbon atoms, or a polyoxyethylene polyoxypropylene glycol containing about 80% polyoxyethylene. The polysiloxane can be obtained from Dow-Corning as DC 473 fluid; the glycol can be obtained from BASF-Wyandotte as "Pluronic".

The anti-adhesive is coated onto the batt, either by dipping the batt into an aqueous mixture containing it, or by spraying it onto the unbonded batt from an aqueous dispersion to a level between about 0.03 and 5%, preferably 0.05 and 0.3%, by weight of the anti-adhesive based on the batt. Spray application is preferred for continuous preparation of the batts of this invention. The aqueous dispersion may conveniently comprise 0.1-0.3% of the active ingredient. The batt should be sprayed with water prior to application of the coatings. Wetting aids in application of the coating.

The anti-adhesive coating applied need not be dried, although it can be if desired, for the adhesive binder may be applied immediately thereafter. The adhesive binder is conveniently applied by spraying it on the batt although dipping the batt, while supported between scrims, in a dispersion of the adhesive may be employed. The binder employed is a copolymer of ethylene and vinyl acetate containing 18-40% by weight po-

lymerized vinyl acetate (preferably 25-30%). Suitable aqueous emulsions of them can be prepared as described in U.S. Pat. No. 3,347,811. Preferably, the polymers have molecular weights corresponding to a melt index of less than 50, more preferably from about 1 to about 20. (Melt index is determined according to ASTM D1238-modified). Usually about 1-5% by weight surfactant is employed to provide storage-stability to the emulsion. Suitable surfactants include the sodium and potassium sulfates of straight-chain fatty alcohols containing 10-18 carbon atoms. It is usually applied from a 50% solids aqueous emulsion.

After application of the adhesive binder, the batt is dried, usually at 120°-150°C., under the compression required to develop the desired characteristics.

Preferably the coated batts will contain from about 1 to 1.5 percent anti-adhesive based on weight of fiber and about 5 to about 8 ounces of adhesive binder per square yard of batt.

The invention is further described in the following Example which is representative thereof and is not meant to be limiting. In the Example, parts are by weight unless otherwise noted.

### EXAMPLE I

Microcellular, closed-cell filaments are prepared substantially as described in Example IV in U.S. Pat. No. 3,381,077. In this procedure, a solution of a high molecular weight ethylene terephthalate polymer in methylene chloride is extruded to yield microcellular closed-cell filaments in which the cells are in a collapsed state.

The filaments are cut to approximately 3-inch (7.6 cm) staple and inflated by brief contact with methylene chloride and perfluorocyclobutane and rapid drying to eliminate the methylene chloride (plasticizer) and to trap inside the cells part of the perfluorocyclobutane (to which the cell walls are impermeable in the absence of the plasticizer).

The inflated filaments are heated in air to about 150°C, which further inflates the cells by air, yielding microcellular, inflated closed-cell pneumatic fibers having a density of about 0.226 g/cc.

Several batts are made of the fibers by wetting them with water and depositing them randomly on a continuous, perforated belt to form a loose batt of about 4 inch (10.2 cm) thickness. In Sample A, no anti-adhesive is employed and the batt sample is used as a control. The

sample is sprayed with a 50 percent solids aqueous emulsion of a 75/25 copolymer of ethylene and vinyl acetate. The sprayed batt is dried at 120°-150°C. and compressed to  $\frac{1}{2}$  inch thickness by calendering. The batt is cooled by circulating air at room temperature before being released from compression. The resulting batt had a density of about 0.032 g./cc. and consists of about equal weights of fiber and binder.

In Samples B and C, the anti-adhesive described in Table I was applied to the batt by adding it to the aqueous emulsion described for Sample A and applying as described for Sample A. The batts were compressed as described for that Sample.

In Samples D, E and F the anti-adhesive described in Table I was applied to the batt by spraying it on from 0.5%, 0.1% and 0.05% solutions, respectively, in water. The aqueous emulsion described for Sample A was then applied and the sample subjected to the drying and compressing described as for Sample A.

In Samples G, H and I, the batts were sprayed with the aqueous emulsion as described for Sample A, and then sprayed with the anti-adhesive described in Table I, as described for Sample D.

Table I shows the results when the sprayed batts A-I were tested for their noise level by the test described as follows:

A wooden box having the overall dimensions of a 1-foot cube with the top open is used to house a microphone (Type 1560-2131, No. 26845). The output of the microphone is fed to a Type 1560-P-40 preamplifier, and thence to a Sound-Level Meter Type 1565-A and a Graphic Level Recorder Type 1521-B. A Sound-Level Calibrator Type 1562 is employed to assure a uniform base level for all tests. (The foregoing equipment is manufactured by General Radio Co.).

A 12 inches  $\times$  12 inches (30  $\times$  30 cm.) sheet of the batt sample is clamped onto the open top of the box; the sound equipment is actuated and a 12-pound ball or metal hemisphere, rounded side down, about 4 inches in diameter is brought into contact with the center surface of the batt, rested thereon and then released slowly. The above-described equipment is capable of measuring, and/or recording, in decibels (db), the volume of any sound which is detectable by the human ear. The background noise in the test room is also measured and the test reading is corrected for this background in the tabulation of results.

TABLE I

| Sample Batt | Anti-Adhesive | Wt. On Fiber | How Added To Sample Batt             | Noise (db) |
|-------------|---------------|--------------|--------------------------------------|------------|
| A           | None          |              | —                                    | 33 or more |
| B           | DC-473        | (1%)         | Added to Adhesive Emulsion           | 22         |
| C           | "Avitone" A   | (5%)         | Added to Adhesive Emulsion           | 21         |
| D           | DC-473        | (0.08%)      | Sprayed on batt before adding binder | 24         |
| E           | DC-473        | (0.40%)      | Sprayed on batt before adding binder | 16         |
| F           | "Pluronic"    | (0.80%)      | Sprayed on batt before adding binder | 18         |
| G           | DC-473        | (0.5%)       | Sprayed on already bonded batt       | 30.7       |
| H           | DC-473        | (1%)         | Sprayed on already bonded batt       | 31.4       |
| I           | DC-473        | (2%)         | Sprayed on already bonded batt       | 32.0       |

DC-473 is a polyoxyethylene, polyoxypropylene polymethylsiloxane obtainable from the Dow Chemical Company. Pluronic F38 is a polyoxyethylene polyoxypropylene glycol obtainable from Wyandotte Chemical Company. "Avitone" A is a sodium alkylsulfonate obtainable from E. I. du Pont de Nemours and Company.

Subjective evaluation indicates that the noise of flexing becomes objectionable above the level of about 27 decibels. Thus, as evidenced by the data in Table I, spraying the anti-adhesive onto an already bonded batt does not provide adequate reduction of noise level.

The preceding representative examples may be varied within the scope of the present total specification disclosure, as understood and practiced by one skilled in the art, to achieve essentially the same results.

The foregoing detailed description has been given for clearness of understanding only and no unnecessary limitations are to be understood therefrom. The invention is not limited to the exact details shown and described for obvious modifications will occur to those skilled in the art.

The embodiments of the invention in which an exclusive property or privilege is claimed are defined as follows:

1. A process for reducing the noise in compressible fibrous structures when flexed under stress, which comprises:

spraying a reticulated batt of randomly arranged, mi-

crocellular, inflated closed-cell, pneumatic fibers of a synthetic organic polymer with between about 0.03 to about 5 percent by weight based on the weight of the fibers of an anti-adhesive comprising an aqueous dispersion of a compound selected from the group consisting of a polyoxyethylene polyoxypropylene polymethylsiloxane containing about 51% polyoxyethylene, a sodium alkylsulfonate of 22 to 24 carbon atoms and a polyoxyethylene polyoxypropylene glycol containing about 80% polyoxyethylene;

coating said sprayed batt with an adhesive binder comprising an aqueous emulsion of at least 40% by weight of an ethylene/vinyl acetate copolymer wherein the vinyl acetate comprises 18-40% by weight of the polymer; and drying the coated batt.

2. The process of claim 1 wherein the synthetic organic polymer is polyethylene terephthalate.

3. The process of claim 1 wherein the anti-adhesive is the polymethylsiloxane described therein.

4. The process of claim 3 wherein the amount of the polymethylsiloxane coated onto the batt is between about 1 and about 5 percent by weight, based on the weight of the fibers.

5. The process of claim 4 wherein the synthetic organic polymer is polyethylene terephthalate.

\* \* \* \*